

Aug. 17, 1943.

O. M. OTTE

2,327,209

ALLOY STEEL ARTICLE AND PROCESS OF PRODUCING THE SAME

Filed May 23, 1941

2 Sheets-Sheet 1



INVENTOR  
Otho M. Otte  
BY  
Evans & Meloy  
ATTORNEYS

Aug. 17, 1943.

O. M. OTTE

2,327,209

ALLOY STEEL ARTICLE AND PROCESS OF PRODUCING THE SAME

Filed May 23, 1941

2 Sheets-Sheet 2



Fig. 7



Fig. 8



Fig. 9



Fig. 10



Fig. 11



Fig. 12

INVENTOR  
Otho M. Otte  
BY  
Evans & McCoy  
ATTORNEYS

## UNITED STATES PATENT OFFICE

2,327,209

ALLOY STEEL ARTICLE AND PROCESS OF  
PRODUCING THE SAME

Otho M. Otte, Tarentum, Pa.

Application May 23, 1941, Serial No. 394,871

3 Claims. (Cl. 29—18)

This invention relates to rolled steel articles and to a method of preparing the same. It particularly relates to alloy steel ingots, bars, slabs, and the lighter sections of sheets, strip and plates, and to the method of preparing the same.

In the preparation of rolling articles as above mentioned, it frequently happens that relatively small pieces or areas of the surface of the steel or metal when in a hot state, become partly separated from the main body of the metal at one or more points and the rolling pressures cause these surface segregations to curl up, fold back or spread out thinly. Since these pieces are but partially attached to the main body of metal, they appear like shingles or chips on the surface of the metal. Such separation occurs during the back and forth rolling operations, and especially is this fracturing of the surface likely to occur during the deformation of ingot into bloom, slab or bar. Once chipping starts, the number of chips or defects are progressively enlarged or areas increased in the further rolling of the metal, so that a very serious surface problem results.

Heretofore, once the surface of the metal ruptured, scaled, laminated or chipped to any appreciable extent, it was necessary to subject the whole mass to an expensive refinishing of surface by grinding or similar operation, during which sufficient metal was removed to present a smooth surface for subsequent rolling.

Surface fracture and similar defects created during rolling deformation, are most noticeable in steels containing substantial quantities of hardening elements, and particularly in alloy steels, which have substantial toughness and hammer-weld with difficulty, or in such steels which do not hammer-weld, especially those containing chromium, molybdenum, nickel or the like.

It is the object of the present invention to provide a method for rolling steels wherein the amount of surface defects and the frequency of their occurrence is largely reduced through rolling technique.

It is a further object of the present invention to provide a steel having modified grain structure and improved characteristics obtained by perfected grain orientation in combination with annealing temperatures best suited to develop the particular physical properties sought.

It is a further object of this invention to provide steel in sheet or strip form having improved surface characteristics, and improved tensile strength.

Other objects will be apparent from the following description of the invention as illustrated in the accompanying drawings, in which:

Fig. 1 is a schematic elevational view showing the steps of the first pass of a suitable ingot through the cogging or blooming mill;

Fig. 2 is a schematic view showing the positions occupied by the metal during the second pass through the cogging or blooming mill;

Fig. 3 is a further diagrammatic view showing the position occupied by the ingot in the third or subsequent passes through the mill rolls to form a slab or bar of the desired shape;

Fig. 4 is a diagrammatic view showing one section cut from a bar or slab in such a manner as to readily designate the proper entry end for further operations;

Fig. 5 is a diagrammatic elevational view of the metal of Fig. 3 during further steps in its reduction;

Fig. 6 is a diagrammatic view showing flow lines of the metal during reduction between the rolls;

Fig. 7 is a diagrammatic view showing the relative movement of the various portions of the metal of Fig. 6 when it is further reduced by rolling it in the same longitudinal direction or sense as in Fig. 6;

Fig. 8 is a diagrammatic view showing the relative movement of the various portions of the metal of Fig. 7 when it is given one pass in the opposite direction;

Fig. 9 shows a portion of an unrolled piece of steel of a single crystal thickness and shows a hypothetical arrangement of the grain crystals separated by impurities, eutectic, or the like;

Fig. 10 illustrates a portion of steel of Fig. 9, showing the effects on the crystal shapes of one or two passes in a single sense;

Fig. 11 illustrates the metal of Fig. 10 after it has been given one or two passes in the reverse direction, showing the effect of the reverse rolling on the structure of the grains; and

Fig. 12 illustrates steel of Fig. 10 which has been reduced entirely in a single sense according to the present invention.

In my prior application, Serial No. 275,696, filed May 25, 1939, now Patent No. 2,260,397, dated Oct. 28, 1941, of which the present application is a continuation-in-part, I disclosed a method for producing silicon steel sheets or strips having improved magnetic properties by rolling them from ingot to final thickness in a single sense, that is, by reducing the metal of the ingot to the desired thickness by rolling it in a single longitudinal direction by always entering the

same end of the metal being rolled into rolls when obtaining effective elongation.

It has now been found that not only silicon steel but that other steels, particularly those containing chromium, molybdenum and nickel, or appreciable quantities of other hardening elements, and the stainless steels, also have improved properties and improved crystal structures. They have greater strength and improved surface characteristics when they are rolled from ingot to slab in the same manner as described in my prior application for silicon steel.

According to the present invention, the metal cast in the form of an ingot is reduced in the blooming mill and in subsequent mills, but each pass is made unidirectionally, i. e., in the same sense. Thus, if the end of the ingot first presented for reduction to the blooming mill is designated A, and the opposite end is designated B, the metal of the ingot is always introduced for reducing passes through subsequent reducing rolls in the direction of A to B, so that it passes therethrough in the same sense, i. e., from A to B. The back and forth rolling of the metal even in the blooming mill affects the grain arrangement and crystal structure in the final article to such an extent that the highest tensile strength and best oriented grain structure is not obtained.

In this application the term "sense" is being used to mean in one longitudinal direction. In other words, in the making of reducing passes, to reduce the metal from the ingot to the desired final thickness, the ingot, slab, bar, sheet or strip, as may in turn be prepared, is presented to the rolls in the same relative position end-to-end as the original ingot was first presented to blooming mill rolls.

Referring to the drawings, the ingot I of steel, which has been stripped in the usual manner from the ingot mold and reheated in the usual manner in a soaking pit to obtain a uniform temperature throughout, and having end portions A and B, respectively, is passed between the rolls 1 and 2 of the blooming mill to elongate it as desired to form the reduced ingot M having end portions A and B, corresponding with portions designated A and B of the ingot. The metal M is then returned to the position shown in Fig. 2, so that the end A may again enter the bite of the rolls 1 and 2 of the blooming mill. The return of the metal M from the position of Fig. 1 to that of Fig. 2 may be accomplished by raising roll 1 of the blooming or cogging mill to allow a dead pass of the metal M therethrough, and using the table rolls to cause the metal to return to the initial position. If the metal is caused to pass through the rolls 1 and 2 in a sense from B to A, all pressure should be removed from the rolls, so that no reduction of metal takes place. Other suitable means, such as providing a shunt or by-pass around the blooming mill, may be used to ensure the presentation of the proper end of the metal to the rolls.

The elongated metal M may be further passed between the rolls 1 and 2 a suitable number of times to produce the bloom P of Fig. 2, and the bloom may be reduced by further hot rolling between the rolls 1' and 2' to the slab S of Fig. 3, or to a bar of suitable size, if desired, having end portions A and B which respectively correspond to the end portions A and B of the ingot.

It is to be noted that, in all passes through the rolling mills after the hot ingot has been initially introduced into the first hot roll mill, a

reduction in thickness of the metal is caused when the end portion A of the metal first enters the rolls and the metal passes therethrough in a sense from A to B.

5 During the rolling operations the metal may be trimmed in the usual manner and, if the quantity of metal is too great for further handling, the slabs S or the bar, as the case may be, may be cut as desired into sections of the desired size or weight. In such cases, however, it is desirable to designate the end portions A and B of the various sheared sections, to make it easy for the operator to determine the proper end of each section of the slab or bar to be introduced into the rolls, so that subsequent reduction takes place in the sense of A to B.

The slab or bar S, diagrammatically indicated as S in Fig. 3, may be further reduced to produce the desired form of metal sheet or metal strip.

20 If it be desired to make a sheet from the slab S, the slab is cut into sections of the desired size and the end portions are marked so that they may be identified as mentioned above, in order that the sections may be rolled longitudinally in 25 the same sense as the original ingot was rolled, i. e., from A to B.

The slab S is particularly adaptable for the rolling of long strips of metal. To accomplish this, the slab S, if large, may be divided into sections of the proper size or weight to give the desired length of a strip of given width and thickness.

In cutting the slab S into sections of the desired weight it is preferable to have the cut so made 35 that the cut itself will designate the A and B ends of the sections. This can be accomplished in various ways, a very convenient method of doing it being to use a wide angle V-shaped shear blade which will give the B end of the section the 40 appearance of what is frequently termed a "fish tail," and the end A is slightly pointed, so that any operator may readily see by inspection the pointed end of the section, which is the one to be entered in the roll. Furthermore, as the rolling 45 proceeds from this point on to the long strip, this marking by the shear is not obliterated through any rolling process.

In Fig. 4 the bar S is shown as having a section cut therefrom, the cut s being in the form of a wide angle V, the pointed end being designated A, and the other end B.

The material from the rolls 1' and 2', which has been reduced to a suitable size and shape, is then further reduced through rolling mills. For example, a stand of three or more pairs of rolls, 55 having proper screw reduction, may be used in line, if desired. In such rolling operations, wherein any reduction in thickness takes place, the end portion designated A is the one entered between the rolls.

60 The slab or bar S is received from the slabbing mill at relatively high temperature, and subsequent heating is usually unnecessary before it is presented to the continuous hot rolls. As shown in Fig. 5, there are three pairs of reducing rolls. The rolls 3 and 4 are preferably spaced so as to produce a relatively high reduction in the thickness of the bar S, and rolls 5 and 6, and 7 and 8, are preferably spaced so as to provide a medium reduction and a low reduction, respectively, in the thickness of the strip material.

65 The relative speeds of the rolls 3 and 4, 5 and 6, and 7 and 8, are preferably adjusted to compensate for the elongation produced, and during the 70 rolling procedure the material may be passed

through suitable normalizing zones, pickling baths, etc., as is apparent to those skilled in the art, and further reduced by hot or cold rolling if desired.

It is contemplated that the metal be normalized or heat treated at suitable points intermediate the rolling operations to maintain its temperature at the desired value. If the material from the continuous hot mill is of suitable thickness for use, it may be wound upon a form having the desired shape, such as that of a coil.

Effects of unidirectional rolling, or rolling in one sense, and effects of back and forth rolling are diagrammatically illustrated in Figs. 6 to 12 of the drawings. In Fig. 6 the unrolled ingot metal 18, having vertical identifying lines 19 thereon, which are spaced uniformly so that flow of the metal may be indicated, is shown as the ingot is passed between reducing rolls 16 and 17 in a direction from A to B to reduce its thickness. The straight identifying lines become curved, as shown at 19a. In Fig. 7 the metal which was reduced in Fig. 6 is shown when given a further reduction in the same sense. It may be seen that this further reduction causes the flow of the metal to continue in the same relative direction as in Fig. 6, with the result that the flow lines 19a become more sharply curved, as shown at 19b, and this becomes more pronounced on further reductions.

In Fig. 8 is illustrated metal from Fig. 6, which is reduced to the same extent as in Fig. 7, by rolling it in the opposite sense. The flow lines 19a become distorted and reversed, as at 19c, showing a reversal of flow of the metal, which destroys the most desirable crystal shape with resulting inferior properties.

Thus, Figs. 6 and 7 diagrammatically indicate the movement of metal when subjected to compression rolls in two rolling operations. From the rolling of the ingot to the finished strip, however, there are usually more than fifteen or more such passes and as such passes are made while the metal is hot, the repeated elongations of the metal in the same sense tend to produce a more uniform crystal axis orientation or grain arrangement. Such crystal axis orientation or grain arrangement seems to be characteristic of metal treated in this manner, and such metal possesses very desirable finish and improved strength in the direction of the grain or rolling.

Fig. 8 illustrates the detrimental effects of a single pass back and forth, which obviously tends to cause a non-uniform or heterogeneous structure, and such structure is emphasized when further back and forth passes are made, resulting in less desirable properties.

Although it is known that even thin sheets or strips of steel usually have a thickness greater than the thickness of a single grain, it is believed that the reason for the improvement obtained by applicant can best be explained by considering the effects of rolling in a single direction and the rolling back and forth on a hypothetical sheet having a thickness of one grain, as is illustrated in Fig. 9. The effects on the metal of such thickness are representative of the effects on thicker metal and the drawing is much simplified.

In Fig. 9 the grains G are shown prior to rolling of the steel, separated by the usual slag, impurities, or other ingredients designated 25, and usually present between the boundaries of the separate grains of the metal. When the grains of Fig. 9 are given a single pass through the re-

ducing rolls they will have substantially the shape of the grains shown in Fig. 10, characterized by the elongated portions of the grains continuously converging towards the ends thereof. If the partially reduced steel of Fig. 10 is now further reduced in the same sense instead of by back and forth reduction, as has always been the practice heretofore, the tongue X of Fig. 10 will be further elongated in length, as shown in Fig. 12, so that the grains are characterized by the elongated portions continuously converging toward their ends, with the grains being oriented and having a sharply curved edge. If the partially reduced steel of Fig. 10 is now rolled in the reverse direction, the metal of the tongue X flows in the opposite direction to the previous flow and the general thickness of the tongue is increased in the vicinity of Y, so that the grains have substantially the form shown in Fig. 11, and although reduced in thickness they are less pointed, shorter and generally of a flatter shape than when they are rolled entirely in a single sense, as were the grains of Fig. 10. Such reciprocally rolled grains do not continuously converge toward their ends. Although the reduction of the metal is the same in Figs. 11 and 12, it is readily seen that the grains of the metal rolled in a single sense are much longer in the direction of rolling than are the grains in the metal of Fig. 11.

It is well known that steels, such as bolts, rods, etc., which are rolled in a back and forth direction without crosswise rolling are much stronger in the direction of their rolling than in the perpendicular direction. This is undoubtedly due to the fact that the grains in steel so produced are elongated solely in the direction of rolling. It is found in accordance with the present invention that the tensile strength is still further improved. Probably this improvement takes place for the same reason, as it will be readily seen, that since the grains are elongated still more when all the rolling, including that of the blooming mill, is in the same sense.

It has also been found that since the grains in the steel produced according to the present invention have greatly increased inter-grain adhesion surfaces with the length of grain face oriented to the common line of elongation and in the same sense, that the mass presents greatly increased resistance to parting or rupture, which break or fracture occurs along the boundary lines between grains, and therefore forces of stretching or tensile force applied parallel to the axis of rolling elongation may be materially increased over like metal and mass that has been formed by first rolling in one direction and then again rolled in the opposite direction. On the surface of the metal there is less of the individual grain body exposed and these grains are accordingly more firmly interlocked with each other and the next underlying surfaces. When the elongation of the metal is in one sense, as above explained, any thin ends of crystals or grains terminating at the surface of the metal are elongated from their point of strongest attachment and at no time are these ends forced in the direction of such point of strongest attachment. There is, therefore, no appreciable tendency for scuffing the ends from the main body of metal and so-called shingling or chipping, which occasionally causes so much havoc in the preparation of molybdenum steels including armor plate, and in the preparation

of other low silicon alloy and stainless steels, is reduced and usually entirely eliminated.

As the heavier reductions in thickness usually take place in the blooming or slabbing mills, a reverse pass on these mills is usually more deleterious to the properties, in that such reverse passes seem to disturb the crystal axis orientation of the resultant strip or sheet to a greater degree than passes in which light reductions of the metal are made. It is, therefore, desirable that nearly all the passes in which substantial reductions are made be in the same sense as the first rolling of the ingot.

After the metal has been reduced to a slab or bar of a suitable thickness for further processing into a sheet or strip the reductions in thickness for a given rolling pass are, of course, considerably less in amount than those for forming the slab or bar. Even in the further processing, the metal should be rolled in a single sense to obtain the best properties, and particularly for the heavier reductions in thickness.

In the reduction of the steel as above described, it is contemplated that it be given coatings of insulating material, such as magnesium oxide, before it is coiled. It is also contemplated that, after the steel has been reduced to a suitable thickness, several laminae of the material may, if desired, be superimposed and given the final reduction in the superimposed condition to produce sheet or strip.

In my above-designated, copending application, now Patent 2,260,397, I disclosed a process for producing relatively thin silicon steel of improved magnetic properties. "Silicon steel" is defined in "Chamber's Technical Dictionary," published by The Maximilian Company of New York in 1940, on page 770, as: "Iron or low carbon steel to which 0.75-4.0% silicon has been added." It is not my intention to claim herein silicon steel according to the above definition.

The principles of the present invention may

be utilized in various ways, numerous modifications and alterations being contemplated, it being understood that the embodiments shown in the drawings and described above are given merely for purposes of explanation and illustration, without intending to limit the scope of the claims to the specific details disclosed.

What I claim is:

1. A process of forming molybdenum steel wherein the amount of surface chipping is substantially reduced, which comprises reducing a molybdenum steel ingot to the desired form by rolling it in a single longitudinal direction by always entering the same end of the metal being rolled into the rolls when obtaining effective elongation, whereby molybdenum steel having all effective elongation in a single sense is produced.
2. A process for producing alloy steels other than silicon steels containing at least one member of the group consisting of chromium, molybdenum and nickel, in which process the amount of surface chipping is substantially reduced, said process comprising casting an ingot of the desired metal, and reducing the metal of the ingot to the desired thickness by rolling it in a single longitudinal direction by always entering the same end of the metal being rolled into the rolls when obtaining effective elongation, whereby alloy steels having all effective elongation in a single sense are produced.
3. A molybdenum steel article substantially free from surface chipping, having the grains of metal elongated in a single longitudinal direction by always entering the same end of the metal being rolled into the rolls when obtaining effective elongation, said article being characterized by having the elongated portions of the grains continuously converging toward the ends thereof, the ends being sharply curved.

OTHO M. OTTE.